

# UNITED STATES PATENT OFFICE.

ROYER LUCKENBACH, OF BROOKLYN, NEW YORK, ASSIGNOR TO LUCKENBACH PROCESSES, INC., OF SAN FRANCISCO, CALIFORNIA, A CORPORATION OF NEVADA.

## PROCESS OF CONCENTRATION OF ORES.

1,417,262.

Specification of Letters Patent. Patented May 23, 1922.

No Drawing.

Application filed January 3, 1921. Serial No. 434,758.

To all whom it may concern:

Be it known that I, ROYER LUCKENBACH, a citizen of the United States, and a resident of the borough of Brooklyn, county of 5 Kings, city and State of New York, have invented a certain new and useful Process of Concentration of Ores, of which the following is a specification.

The invention relates the concentration 10 of ore in which the mineral values are separated from the earthy or rocky gangue of the ore by flotation whereby the valuable mineral content of the ore will be caused to float upon the surface of a pulp formed 15 of finely divided ore and water, and the gangue will not be so floated but will sink in the water.

The flotation processes at present in use 20 are applicable generally to the recovery of metallic sulphides, and in most cases it is necessary for efficient working, that the pulp be acidified, and in some situations the pulp must be heated. Such prior processes will 25 not successfully float carbonate, oxides and silicates of the metals.

The objects of the present invention are 30 to produce a process whereby mineral values may be separated from the earthy or rocky gangue constituents of the ore and floated on the surface of the pulp; to provide a frothing and mineral selecting process characterized by the absence of free oils and greases in the mixture employed in the pulp; to provide a process wherein mineral 35 carbonates, oxides and silicates, as well as free metals and the sulphides of such metals will be separated from the gangue; to provide a frothing and gathering process wherein certain non-metallic minerals, such 40 as graphite and sulphur, may be separated from their gangue, and for producing a compound having highly efficient frothing properties without reducing the mineral gathering 45 qualities thereof.

These and further objects will more fully appear in the following specification and claims.

The invention consists in the mixing of 50 finely divided ore with water to form a pulp, to which is added a small quantity of a reagent comprising a liquefied resin or combination of resins. The resin or resins may be liquefied by means of an alkali, or alcohol, and may be combined with the reaction

product of an alkaline metal and a fatty 55 acid. The reagent may if desired be employed in conjunction with a normally unsaponifiable oil or oily substance, in which case the reagent will act as a frother while at the same time it will supplement whatever mineral gathering properties the oil or oily substance may possess.

The preferred resin for use in compounding the reagent is lac, and the same may be used in any of its commercial forms, such 65 as seed lac, stick lac or shellac. The preferred fatty acid is oleic acid, and the preferred alkali is caustic soda. Ammonia may be employed instead of or in conjunction 70 with the caustic soda.

The lac may be liquefied in alcohol before 75 being mixed with the other ingredients, and in some situations, and with certain ores, it is desirable that an excess of alcohol be employed.

The fatty acid is not present as such in the mixture but is in a neutralized form such as sodium oleate. The resin in the reagent, at least, is in neutralized form because of the presence of the alkali.

The preferred reagent is composed of a mixture in which water, lac, caustic soda, alcohol, and oleic acid are employed. When the mixture is completed it comprises the diluted reaction product of lac and alcohol, 85 and the reaction product of oleic acid and caustic soda, the reagent as a whole having an alkaline reaction.

The reagent may be compounded in the following proportions: Water 85 cc., alcohol 90 15 cc., shellac 5 grams, caustic soda 2.5 grams and sodium oleate 5 grams. In a test on a Utah copper "capping" carbonate ore, containing a small percentage of sulphide, in a Janney laboratory machine the following 95 result was obtained:

| Product.          | Wt. grs. | Assay per cent. Cu. | Gr. Cu contained. | Per cent. of total Cu contained. |
|-------------------|----------|---------------------|-------------------|----------------------------------|
| Feed.....         | 500.0    | .78                 | 3.90              | 100.0                            |
| Concentrates..... | 38.6     | 3.78                | 1.46              | 37.4                             |
| Middlings.....    | 71.8     | 1.26                | .90               | 23.1                             |
| Tails.....        | 386.4    | .38                 | 1.47              | 37.5                             |
|                   | 496.8    | .....               | 3.83              | 98.0                             |
|                   |          |                     |                   | 105                              |

In a test run on the same ore and under the same conditions but with a reagent com-

pounded with water 100 c. c., sodium oleate 5 gr., shellac 5 gr., caustic soda 2½ gr., the following result was secured:

| 5  | Product.          | Wt. gr. | Assay per cent. Cu. | Gr. Cu contained. | Per cent. of total Cu contained. |
|----|-------------------|---------|---------------------|-------------------|----------------------------------|
| 10 | Feed.....         | 500.00  | .79                 | 3.95              | 100.0                            |
|    | Concentrates..... | 16.4    | 4.97                | .82               | 20.8                             |
|    | Middlings.....    | 76.0    | 1.65                | 1.25              | 31.7                             |
|    | Tails.....        | 403.8   | .38                 | 1.53              | 38.8                             |
|    |                   | 496.2   | .....               | 3.60              | 91.3                             |

In the above tests the ore was crushed to 15 80 mesh, the dilution was 4 to 1, and the water was Brooklyn tap water, and the time was 15 minutes. The froth which was raised in the first five minutes is the "concentrates," the rest is the "middlings."

20 The lac-alcohol solution, when used, is preferably made by dissolving 6 oz. of lac in 1 gallon of alcohol. Alcohol in addition to that of the lac solvent may be employed in the mixture.

25 The sodium oleate and the sodium resinate form a perfect emulsion and the reagent is free of oil and acid, and is not actively acid in its effects on the mineral content of the ore. The reagent has a particular affinity 30 for the sulphides, carbonates and oxides of nearly all minerals in practically every form in which such minerals are found in nature. The reagent will select and float the mineral values resulting in great economy of operation.

35 In operating on sulphide ores a reagent compounded of water, an alkali, and lac, which latter may have been previously dissolved in alcohol, or a mixture formed of 40 water, oleic acid and an alkali may be used. Either of the above reagents will form a perfect emulsion. There will be no free oil or free acid in the mixture. A strong, free flowing froth will be formed, and this froth 45 will float sulphides as well as free metals.

In working certain ores, or certain grades of the same ore, or ore of certain fineness some of the ingredients may be omitted.

The following reagents may be used:

50 1. Water, and the reaction product of caustic soda and oleic acid.

2. Water, and the reaction product of caustic soda and lac.

3. Water, and the reaction product of 55 caustic soda and shellac and alcohol solution.

4. Water, the reaction product of caustic soda and a fatty acid, and the reaction product of caustic soda and shellac.

60 5. Water, the reaction product of caustic soda and a fatty acid, and shellac and alcohol solution.

6. Any of the above reagents with the addition of ammonia.

65 Instead of caustic soda other alkalies, such

as sodium carbonate, may be employed, or borax may be used.

The alkali saponifies the fatty acid, and the lac, and each intensifies the selective qualities of the other.

70 The ingredients of the frothing and mineral selective agent are given as types and are not intended to form an exhaustive list of substances suitable for the purpose.

The proportions of the various ingredients 75 of the reagent may vary within wide limits, depending on the character of the ore to be worked and on other conditions, and more or less be supplied to the pulp as required.

The reagent may, if desired, be made up 80 in separate batches and be placed in the pulp separately. The operator will thus have complete control of the process. The proportions of the various ingredients may thus be varied as the operating conditions 85 vary.

In operation, a pulp of ore and water of the proper fluidity is placed in a flotation apparatus and thoroughly aerated, preferably by agitation. The reagent is admitted 90 to the pulp and because of the aeration will form bubbles throughout the pulp. The mineral constituents of the ore will adhere to the bubbles and be floated to the surface of the pulp while the gangue will not so 95 adhere and will sink to the bottom of the apparatus. The mineral bearing froth may be removed from the surface of the pulp, and the values are separated from the reagent in any desired manner.

100 The water may now be separated from the gangue, as by settling, and reused to form a new pulp, and because of the presence of some, at least, of the ingredients of the reagent remaining therein, lesser amounts of 105 those substances need be supplied to the new pulp.

The values may be released from the reagent of the froth, in part at least, by settling or pressing after the bubbles have been 110 broken, and the reclaimed reagent be reused.

Instead of placing the reagent in the pulp as above described the same may be added to the water before the pulp is formed.

115 By means of the present process not only free metals and their salts may be gathered and floated, but certain non-metallic minerals, for example, graphite, sulphur and their chemical compounds may be recovered. Any mineral substance which is essentially 120 water repellent, and will not be wetted by water, may be floated.

This application is a continuation in part of applicant's application entitled Concentration of ores, filed August 16, 1917, and 125 numbered serially 186,642.

In accordance with the provisions of the patent statutes, the principle of the invention has been described together with what is now considered the best embodiment there- 130

of, but it is desired to have it understood that the embodiment described is merely illustrative, and that the invention may be carried out in other ways.

5 Having now described the invention what is claimed and desired to be secured by Letters Patent is as follows:

1. The process of concentrating ores, which comprises adding to a pulp composed of 10 finely divided ore and water the reaction product of an alkali and lac, aerating the mixture to form a froth, and separating the froth from the remainder of the pulp.

2. The process of concentrating ores, which 15 comprises adding to a pulp composed of finely divided ore and water the reaction product of an alkali and lac and alcohol, aerating the mixture to form a froth, and separating the froth from the remainder of 20 the pulp.

3. The process of concentrating ores, which comprises adding to a pulp composed of 25 finely divided ore and water the reaction product of caustic soda and lac, aerating the mixture to form a froth, and separating the froth from the remainder of the pulp.

4. The process of concentrating ores, which comprises adding to a pulp composed of 30 finely divided ore and water the reaction product of caustic soda and lac and alcohol, aerating the mixture to form a froth, and separating the froth from the remainder of the pulp.

5. The process of concentrating ores, 35 which comprises adding to a pulp formed of finely divided ore and water the reaction product of an alkali, lac and ammonia, aerating the mixture to form a froth, and separating the froth from the remainder of 40 the pulp.

6. The process of concentrating ores, which comprises adding to a pulp formed of 45 finely divided ore and water the reaction product of a caustic alkali, lac and ammonia, aerating the mixture to form a froth, and separating the froth from the remainder of the pulp.

7. The process of concentrating ores, which 50 comprises adding to a pulp formed of finely divided ore and water the reaction of caustic soda, lac and ammonia, aerating the mixture to form a froth, and separating the froth from the remainder of the pulp.

8. The process of concentrating ores, 55 which comprises adding to a pulp formed of finely divided ore and water the reaction product of an alkali, lac dissolved in alcohol and ammonia, aerating the mixture to form

a froth, and separating the froth from the remainder of the pulp.

60

9. The process of concentrating ores, which comprises adding to a pulp composed of finely divided ore and water the reaction product of an alkali, a fatty acid and lac, aerating the mixture to form a froth, and 65 separating the froth from the remainder of the pulp.

10. The process of concentrating ores, which comprises adding to a pulp composed of 70 finely divided ore and water the reaction product of an alkali, a fatty acid and lac and alcohol, aerating the mixture to form a froth, and separating the froth from the remainder of the pulp.

11. The process of concentrating ores, 75 which comprises adding to a pulp composed of finely divided ore and water the reaction product of caustic soda, oleic acid and lac, aerating the mixture to form a froth, and separating the froth from the remainder of 80 the pulp.

12. The process of concentrating ores, which comprises adding to a pulp composed of 85 finely divided ore and water the reaction product of caustic soda, oleic acid and lac, and alcohol, aerating the mixture to form a froth, and separating the froth from the remainder of the pulp.

13. The process of concentrating ores, 90 which comprises adding to a pulp formed of finely divided ore and water the reaction product of an alkali, a fatty acid, lac, ammonia, aerating the mixture to form a froth, and separating the froth from the remainder of the pulp.

95

14. The process of concentrating ores, which comprises adding to a pulp formed of 100 finely divided ore and water the reaction of caustic soda, oleic acid, lac and ammonia, aerating the mixture to form a froth, and separating the froth from the remainder of the pulp.

15. The process of concentrating ores, which comprises adding to a pulp formed of 105 finely divided ore and water the reaction product of an alkali, oleic acid, lac, alcohol, and ammonia, aerating the mixture to form a froth, and separating the froth from the remainder of the pulp.

This specification signed and witnessed 110 this 31st day of December, 1920.

ROYER LUCKENBACH.

Witnesses:

A. E. RENTON,  
J. F. COLEMAN.